

Sept. 20, 1927.

1,642,778

G. W. ELMEN

RECEIVER

Filed Nov. 4. 1924



Inventor:  
Gustaf W. Elmen

by *Edward A. Edwards Atty*

Patented Sept. 20, 1927.

1,642,778

# UNITED STATES PATENT OFFICE.

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK.

## RECEIVER.

Application filed November 4, 1924. Serial No. 747,718.

This invention relates to receivers, and more particularly, to a diaphragm for use in the magnetic circuit of a telephone receiver.

5 In my copending application Serial No. 492,722, filed August 16, 1921, I have described an electromagnetic device such as a telephone receiver in which at least a portion of the magnetic circuit is composed of 60 a material having very high permeability at low magnetizing forces.

For certain uses I have stated that an alloy containing approximately 78½% nickel and 21½% iron is the most suitable 65 material, but for other uses, this proportion may vary somewhat and in certain cases it may even be desirable to add a third ingredient. In other words, to obtain the best results in a particular case, it is desirable 70 to employ as the magnetic material, an alloy in which the proportion of the ingredients and the heat treatment provided are such as to give the optimum characteristics for 75 that particular use.

25 It is the object of the present invention to increase the sensitivity of an electromagnetic device such as a telephone receiver. This object is accomplished by improving the characteristics of the vibrating diaphragm thereof. In a telephone receiver particularly in one of the electromagnetic type, it is necessary that the receiver be an efficient transducer for converting the electrical energy of the speech currents into 80 sound energy and, furthermore, the maximum efficiency should be realized under the conditions existing on long subscriber loops where the magnetizing current is a minimum and the flux density in the diaphragm 85 is therefore low.

In a receiver of this type, there are two forces which play an important part in determining its characteristics, namely, a variable force resulting from the combined action of the polarizing and the variable flux and a steady force due to the action of the polarizing flux alone. The former constitutes the useful driving force and the latter owing to the control which it exerts 90 over the reluctance of the air gap influences not only the efficiency at small magnetizing currents, but is instrumental in determining the magnetizing current at which maximum efficiency occurs. The magnitude of the 95 steady force resulting from the polarizing

flux at high magnetizing currents, also has an important bearing on the stability of the receiver, since it is influential in determining the minimum separation which may be employed between the diaphragm and 100 pole pieces. On long subscriber loops where the magnetizing current is small and the flux density in the diaphragm is therefore low, the length of the air gap determines 105 the magnitude of the polarizing flux. Therefore, the effective permeability becomes the most important factor in determining the useful driving force. Since the 110 terminal impedances of the receiver considered as a transducer are fixed by the electrical impedance of the apparatus at the subscriber's station and the acoustic impedance of the ear, the number of turns which can be employed in the energizing winding and the mass of the diaphragm are limited. It is necessary, therefore, if the receiver is to be 115 most efficient on long loops and not introduce transition losses of an electrical and mechanical nature that the diaphragm be 120 of low mass and of such a material and thickness that it will approach saturation with the current supplied on long subscriber 125 loops.

In accordance with a feature of the invention a vibrating diaphragm such as a receiver diaphragm is composed of a material which when properly heat treated has a very high effective permeability at low magnetizing forces. Furthermore, the elasticity and other mechanical properties of the material 130 are such as to permit the use of a diaphragm of low mass to meet the requirements of maximum efficiency at low magnetizing forces.

This and other features of the invention will be more clearly understood by reference to the accompanying drawing in which:

Fig. 1 is a sectional view of an electromagnetic receiver embodying the features of 135 this invention.

Fig. 2 is a view of the diaphragm of Fig. 1.

Fig. 3 shows the gain in efficiency resulting from following this invention.

Fig. 4 contains curves showing the variation in effective permeability at different magnetizing forces for various magnetic materials.

Referring more particularly to Fig. 1 the receiver comprises an energizing winding 5 140

mounted on the center leg 6 of an E-shaped pole piece comprising the outer legs 7-7. This pole piece is rigidly secured as by welding to a mounting plate 8, which in turn, is secured to the receiver cup 9. The diaphragm 10 is mounted in operative relation to the pole pieces and is clamped in position by the receiver cap 11 which threads on the cup portion 9.

10 The pole pieces and diaphragm are composed of a magnetic material having an effective permeability at low magnetizing forces very much higher than that of iron, a low hysteresis factor and a resistivity of the 15 order of 45 microhms per cubic centimeter. To obtain this material iron and nickel are fused together in an induction furnace preferably in the proportion of 55% iron and 45% nickel, good commercial grades of these 20 materials being suitable for this purpose. The molten composition is then poured into a mold and cooled either in the form in which it is later to be employed or in a convenient form to be worked over for that purpose. While 55% iron and 45% nickel are 25 mentioned as being the proportion of nickel and iron preferably employed, it should be understood that this proportion may deviate somewhat from these figures. To develop 30 the utmost permeability of this magnetic material, the finished parts are subjected to a heat treatment which in particular cases varies somewhat as regards the temperature employed and the duration of the heating 35 and cooling periods. The optimum values of these variables may be readily determined for a specific case by experiment. In the case of diaphragms the preferred composition consisting of the 55% iron and 45% 40 nickel is rolled into sheets, approximately six thousandths of an inch thick. The diaphragms are then punched from these sheets which may be stretched before the diaphragms are punched therefrom in order to 45 insure perfectly flat diaphragms, or the stretching may be omitted and the completed diaphragms flattened under pressure. The diaphragms are then placed in a container between suitable blocks of lavite or similar 50 material and are heated to a temperature of 1,100° centigrade and maintained at this temperature for a period of one hour, after 55 which, they are slowly cooled. The temperature to which the diaphragms are heated as well as the period during which they are maintained at the high temperature may vary considerably. A temperature as low as 950° C. has been successfully used.

60 Referring to Fig. 3 curve A shows the gain in efficiency expressed in transmission units or miles of standard cable, of an electromagnetic receiver provided with pole pieces of this preferred composition, and a ferro-type diaphragm as compared with a 65 standard type of subscriber's station re-

ceiver. Curve B shows the greater gain in efficiency resulting from also replacing the ferro-type diaphragm with a diaphragm of the preferred composition. It will be noted that not only is the maximum efficiency 70 much higher in the case of the receiver equipped with the nickel iron diaphragm, but this maximum efficiency is attained at a lower magnetizing force corresponding to the conditions present on long subscriber 75 loops.

In Fig. 4 curve A shows the variation in A. C. permeability for a very pure grade of magnetic iron for various superimposed direct current magnetizing forces, and curve B 80 shows the variation in A. C. permeability under similar conditions of an alloy containing 55% iron and 45% nickel when given the preferred heat treatment. It will be noted that for small magnetizing forces of the order of a few tenths of a gauss, which corresponds to the direct current magnetizing force obtainable on long subscriber loops, the effective permeability of the preferred composition is from eight to twelve times 85 that of the high grade magnetic iron. The application of this heat treatment to receiver diaphragms composed of ferro-type metal also results in an appreciable gain in efficiency, but the results are not comparable 90 with those obtained when using the preferred nickel-iron composition.

What is claimed is:

1. The method of making a diaphragm which comprises severing the diaphragm 100 from a sheet of magnetic material, heating said diaphragm to a temperature of the order of 1000° C. and slowly cooling it.
2. A diaphragm composed of nickel and iron heat treated to develop its maximum 105 permeability.
3. A vibrating diaphragm composed of approximately 55% iron and 45% nickel.
4. In a telephone receiver, a magnetic circuit in which the pole pieces and diaphragm 110 are composed of a nickel-iron alloy having a permeability higher than that of iron for low magnetizing forces of the order of those present under operating conditions.
5. In a telephone receiver, a magnetic circuit 115 in which the pole pieces and diaphragm are composed of a nickel-iron alloy having a permeability higher than that of iron at low magnetizing forces and a lower saturation point.
6. In a telephone receiver, a magnetic circuit 120 in which the pole pieces and diaphragm are composed of a magnetic material containing approximately 55% iron and 45% nickel.
7. A vibrating diaphragm having an alternating current permeability higher than that of iron when subjected to a superimposed direct current magnetizing force.
8. A vibrating diaphragm composed of 125

material having a higher effective permeability than iron when subjected to a variable magnetizing force superimposed upon a steady magnetizing force of the order of a few tenths of a gauss.

9. A vibrating diaphragm composed of approximately 55% iron and 45% nickel heat treated to develop a higher effective permeability than iron when subjected to a

variable magnetizing force superimposed upon a steady magnetizing force, and approaching saturation at lower flux densities than iron.

In witness whereof, I hereunto subscribe my name this 3rd day of November, A. D. 1924.

GUSTAF W. ELMEN.